

## UNITED STATES PATENT OFFICE.

LYNDON D. WOOD, OF BALA, PENNSYLVANIA.

## COATING COMPOSITION AND PROCESS.

No Drawing.

Application filed July 1, 1922. Serial No. 572,324.

To all whom it may concern:

Be it known that I, LYNDON D. Wood, a citizen of the United States, residing at Bala, in the county of Montgomery and State of Pennsylvania, have invented new and useful Improvements in Coating Composition and Processes, of which the following is a specification.

This invention relates to compositions for coating surfaces whereby said surfaces under the action of light are rendered sensitive to electric currents and it has more particular reference to a process for making a sensitive compound for use in the reproduction of sound waves which have been photographed upon films or plates.

The object of this invention is the production of the nature hereinbefore referred to which when applied to a surface capable of conducting electric currents renders the same usable for the reproduction of sound waves by the action of waves of light.

My composition consists essentially of a mixture of:

|                                                  | Parts. |
|--------------------------------------------------|--------|
| 25 Platinum-barium-cyanide of potassium crystals | 20     |
| Tungstate of soda                                | 10     |
| Selenium crystals                                | 70     |
| Salt                                             | 34     |
| 30 Sulphur                                       | 33     |
| Phosphorus                                       | 33     |

Although I have specified the proportions above set forth there can be slight modifications thereof without lessening the efficiency and sensitiveness of my composition.

The platinum-barium-cyanide of potassium crystals, tungstate of soda and selenium crystals are thoroughly mixed and brought to a melting point and thereby reduced to a molten mass. To this mass while in its molten state thoroughly I mix the salt, sulphur and phosphorus and again bring this mixed mass to its melting point. This mass is then kept at its melting point by the continued application of heat, for a period of approximately 30 minutes or until a flame rises from the surface of the molten mass of a color indicating the flame of both barium and potassium. At this point the application of heat is discontinued and the mass is then subjected to a sudden cooling by being plunged into a receptacle containing water at a temperature of approximately 40° Fahrenheit.

The resultant composition may be applied to any desired surface by reheating it until it is again reduced to a molten condition into which mass the object or surface to be coated can then be dipped or immersed until a proper coating has been applied thereto, when it can be withdrawn and allowed to cool and harden.

This composite material when applied to any suitable body and exposed to the action of light void of violet rays will affect an electrical current passing through it in accordance with the variation in intensity and character of the light vibrations received by it and therefore has the facility and property of translating light waves and variations therein into electric pulsations and variations thereof. An element so coated by this material composed and prepared as above described is what may be termed a sensitive to light element by which the reproduction of sound waves preferably photographically recorded on a film or plate can be accurately accomplished by electric and electro-magnetic co-operating means.

Having thus described my invention, what I claim as new and desire to secure by Letters Patent is:

1. A sensitive compound for use in the reproduction of sound waves which have been photographically recorded comprising 20 parts of platinum-barium-cyanide of potassium crystals, 10 parts of tungstate of soda, 70 parts of selenium crystals, 34 parts of salt, 33 parts of sulphur, 33 parts of phosphorus.

2. The process of producing a sensitive compound for use in the reproduction of sound waves which have been photographically recorded, consisting in reducing to a molten mass a mixture of platinum-barium-cyanide of potassium crystals, tungstate of soda and selenium crystals and to this molten mass adding a mixture of salt, sulphur and phosphorus and keeping the whole in a molten condition for a continued period of approximately 30 minutes or until a flame color indicating the flame of both barium and potassium rises from the mass and then crystallizing the mass by suddenly immersing it into a receptacle of water at a temperature of approximately 40° Fahrenheit.

In testimony whereof I affix my signature.

LYNDON D. WOOD.